

Aug. 5, 1952

L. F. FIESER  
INCENDIARY GELS

2,606,107

Filed Nov. 1, 1943



*Inventor*  
Louis F. Fieser

*By* Fred S. Lockwood  
*Attorney*

## UNITED STATES PATENT OFFICE

2,606,107

## INCENDIARY GELS

Louis F. Fieser, Belmont, Mass., assignor to the  
United States of America as represented by the  
Secretary of War

Application November 1, 1943, Serial No. 508,632

15 Claims. (Cl. 44—7)

1

The invention described herein may be manufactured and used by or for the Government for governmental purposes without the payment to me of any royalty thereon.

This invention relates generally to gelled fuels and improved gelling agents or thickeners therefor. More particularly, the invention is concerned with the production of new and improved gelled hydrocarbon fuels and gelling agents therefor, for use in incendiary munitions of both the burster and the tail-ejection types, in flame throwers, in hand grenades, in fire starters and, generally, in any incendiary munition which utilizes a combustible liquid or low-melting solid or gelled fuel.

Prior to the present war, rubber was used to thicken or gel gasoline and similar hydrocarbon liquids to make gelled incendiary fillings. However, because of the scarcity of rubber, it has been necessary to resort to and develop other types of gelling agents. This has been a rather difficult problem since the requirements of such incendiary fillings are manifold and exacting. The incendiary gels must be stable and free from syneresis throughout a temperature range from —40° F. to 125° F., since incendiary munitions must be capable of use from the cold regions of Alaska to the tropics. The incendiary gels must have a high inner cohesion so that when they strike a target, they will adhere thereto without falling off so as to do the greatest damage.

It is known that soaps of polyvalent metals, particularly aluminum, are capable of producing gels with both aliphatic and aromatic hydrocarbons. The aluminum soaps which may be used for this purpose are of two main types. One type comprises the group of the aluminum soaps of saturated fatty acids (usually but not necessarily of vegetable origin) as exemplified by the aluminum laurates, palmitates, stearates and myristates. Aluminum stearate has certain disadvantages as a gelling agent for incendiary fuels, both because a heat treatment is required for incorporation into the fuel and because the gels are hard and friable and lack the cohesive and adhesive character desired in an incendiary fuel. Soaps of fatty acids of lower molecular weight, for example, aluminum laurate and myristate, may solvate fairly rapidly at ordinary temperatures but give gels which lack body, which tend to undergo syneresis at low temperatures, and which are of generally inferior quality.

The second type of aluminum soap, as classified with respect to performance in the gelling of hydrocarbons, is exemplified by the aluminum naphthenates and aluminum oleates, these differing from the soaps of the first type in that they are either resinous gums or low-melting solids. As thickening agents for hydrocarbon solvents, the soaps of the second type have the

2

disadvantage that gelation of the fuel is not easily accomplished without either a heat treatment of the mixture or a special processing of the soap. Thus, although a resinous aluminum naphthenate can be processed by alcohol washing to give a product which will solvate at ordinary temperature, the process is costly and the yield is poor. Another method of processing a naphthenate to secure low-temperature gelation is by precipitation as the solid hydroxylaluminum soap. However, the melting point of the resulting product is so low that it may be difficult to avoid agglomeration of the material. As regards aluminum oleates, no prior methods appear to be available for effecting gelation in a simple manner without heating. Furthermore, the aluminum naphthenate and oleate soaps tend to be rather weak, and an excessive amount of soap is required to produce a gel of desired viscosity.

It is evident from the foregoing that aluminum soaps of both the paraffin carboxylate type and the naphthenate-oleate type are subject to certain serious disadvantages and limitations as thickening agents for the production of incendiary gels.

Accordingly, the primary object of this invention, generally stated, is the provision of new and improved gelling agents for producing high-grade incendiary gels or fuels which meet or exceed existing specification and requirements.

A more particular object of this invention is the provision of a new and improved incendiary fuel in the form of a cohesive, elastic, highly-stringy gel that is capable of adhering as a thick mass to walls, ceilings, and even smooth glass surfaces, and which when ignited burns for a relatively long period of time without melting or running, producing a vigorous, highly destructive flame of great incendiary action.

A further object of the invention is the provision of a gelled fuel of the foregoing type further characterized by having the following combination of properties:

(1) Low-temperature coefficient whereby desirable properties are retained over a wide temperature range.

(2) Thermal stability and freedom from syneresis when stored either under tropical conditions or under frigid conditions, or when subjected to cyclic heating and cooling conditions.

(3) Shock stability and freedom from syneresis when subjected to the action of burster charges of the type likely to be employed in incendiary munitions.

Another object of the invention is the provision of a new and improved low-temperature gelling or thickening agent capable of converting any suitable liquid hydrocarbon fuel, such as gasoline (leaded or unleaded), benzene, naphtha, petroleum ether, Stoddard's solvent and diesel oil,

to a gelled fuel of the character described above, by a process which does not require special chemical, thermal or mechanical treatment or equipment.

Still another object of the invention is the provision of a low-temperature gelling or thickening agent, and a process of utilizing the same, which permits the filling of incendiary munitions with gelled fuels under adverse field conditions such as are likely to be encountered in the theatre of operations.

Other objects of the invention will, in part, be obvious, and will in part appear hereinafter.

For a more complete understanding of the nature and scope of the invention, reference may be had to the following detailed description thereof, setting forth by way of illustration certain specific compositions and methods of preparation and utilization, taken in connection with accompanying drawing in which the single figure is a perspective view of a standard wooden structure used in testing the incendiary characteristics of different incendiary gels forming embodiments of this invention.

In accordance with the present invention, it has been found that the foregoing objects thereof may be attained by employing a new and improved composite gelling or thickening agent comprising two or more components suitably combined and incorporated with a hydrocarbon liquid, all as more particularly described and claimed hereinafter.

Broadly speaking, the composite thickener of the present invention comprises two or more components which may be designated and referred to as component A and component B. Component A may comprise an aluminum soap of a soap-forming saturated fatty acid of not more than 15 carbon atoms, and preferably one having from 8 to 14 carbon atoms. Component B may be said to consist generally of (1) a soap-forming carboxylic acid having one or more carbocyclic rings; or (2) a soap-foaming unsaturated fatty acid; or (3) the corresponding aluminum salts of such acids; or (4) any mixtures thereof.

Composite thickeners of the above type have been found to be capable of effecting low-temperature gelation of hydrocarbon liquids generally, producing gelled fuels having the required properties as outlined above.

In preparing the gelled fuels of the present invention, the preferred thickener may be incorporated in any convenient manner with the selected liquid hydrocarbon and the mixture permitted to stand until gelation occurs. However, in some instances, it may be preferable to form a solution of one component of the improved gelling agent (for example, component A), in the fuel to be gelled and thereafter to add the other component or components (for example, component B) to the mixture. In still other instances, it may be desirable to mix the composite gelling agent at an elevated temperature with a portion of the fuel to be gelled and then to blend the resulting homogeneous gummy product with further quantities of the same or different liquid hydrocarbon fuel.

Another desirable method of producing the ultimate gelled fuel is to incorporate the composite gelling agent with a sorbent material (preferably combustible) having a relatively fine state of subdivision, using a sufficient amount of the sorbent material to produce a granular composition which may then be mixed with the hydrocarbon liquid to be gelled. The use of a combustible

sorbent material such as charcoal, flour and the like is particularly advantageous, not only because of the desirable physical properties of the resulting granular material, but also because, unexpectedly, the final gel is characterized by a definitely enhanced incendiary action.

As indicated above component B may consist either of the aluminum soaps of the stated soap-forming acids, or the free acids themselves. In certain instances, it may prove advantageous to employ an aluminum soap for component A and two aluminum soaps, or one aluminum soap and one free acid, or two free acids as component B. Thus for example, the gelling agent may consist of the aluminum soaps of coconut fatty acids (which are characterized by a high lauric acid content) as component A, together with aluminum naphthenate and aluminum oleate, as component B. In short, it will be evident that components A and B do not necessarily consist of pure individual chemical compounds. On the contrary, for economic and other reasons, it is usually preferable to employ mixtures of compounds as the individual components which are rich in the desired ingredients. In this connection it may be mentioned that various acids and soaps, in addition to those identified above, may be present either as adventitious materials included in the components or as deliberately added adjuncts.

As indicated above in characterizing component A, not all soap-forming fatty acids are suitable for producing the improved gelling agent of the present invention. Indeed, selection must be made from the limited group comprising the aluminum soaps of saturated carboxylic acids of not more than 15 carbon atoms and preferably from those having from 8 to 14 atoms inclusive. Lauric acid is a preferred ingredient because of its availability, but this may be replaced by the higher homologue, myristic acid, or by the lower homologues, capric or caprylic acid, or by synthetic saturated acids, for example, 2-ethyl-n-hexoic acid. The common acids having more than 15 carbon atoms, e. g., palmitic and stearic acid, are definitely unsatisfactory, although, as will be shown, substantial amounts of these and other acids outside the C<sub>8</sub>-C<sub>14</sub> range can be tolerated along with components A and B without detracting materially from the quality of the thickener.

There is no restriction with regard to component B, and either the free acids, the aluminum salts or mixtures of either or both may be used. Thus component B may be an aluminum naphthenate, an aluminum oleate, or the aluminum soap of a vegetable or animal oil acid rich in oleic acid but containing as well acids of both higher and lower degrees of unsaturation. If desired, one may employ the aluminum soaps of natural or synthetic acids simulating the properties of either oleic acid or naphthenic acids, for example, acid mixtures obtained by the partial oxidation of petroleum fractions.

Furthermore, the invention is not restricted to the use of single compound for component B, for mixtures of two or more soaps or two or more free acids or an acid and a soap selected from the group may be employed. Nor is there any restriction in the manner in which a selected component is made, for the soaps, for example, may be produced by any of the known methods, including precipitation from an aqueous solution

of the sodium soap or by fusion of the acid with an oxide or hydroxide of aluminum.

Typical formulations for the preparation of thickeners are as follows:

(1)

1 part—aluminum soap of coconut acids  
1 part—aluminum naphthenate

(2)

1 part—aluminum soap of coconut acids  
1 part—aluminum oleate

(3)

2 parts—aluminum soap of coconut acids  
1 part—aluminum naphthenate  
1 part—aluminum oleate

(4)

2 parts—aluminum soap of babassu oil acids  
1 part—aluminum naphthenate  
1 part—aluminum oleate

(5)

2 parts—aluminum laurate  
1 part—aluminum naphthenate  
1 part—aluminum oleate

Several additional satisfactory formulations are indicated in the specific examples given below, and it will be evident that considerable variation is possible with respect to the selection of the ingredients. Within limits, variation is also permissible with respect to the proportions of the ingredients, and the proportions indicated in the examples are typical. While the mean proportions of the ingredients of the thickener are in the neighborhood of equal portions of components A and B, there is a fair amount of latitude possible in the range of percentages of both ingredients which yield satisfactory thickeners and which are within the scope of this invention. In general, a satisfactory thicker will result from a composition having from 1 to 2.5 parts of component A mixed with from 1 to 1.25 parts of component B; this will be clearly shown in the illustrative examples which follow. Within this framework, ranges more limited in scope are best suited for specific ingredients of component A. For example, when component A is the aluminum soap of the fatty acids found in coconut oil, the preferred proportions thereof are from 1 to 1.7 parts. However when component A is the aluminum soap of a saturated fatty acid fraction having from 8 to 14 carbon atoms per acid molecule, the preferred proportions thereof are from 1.5 to 2.5 parts, except when it is combined with the aluminum salt of naphthenic acid as component B. In compositions having the aluminum salt of naphthenic acid as component B the preferred range of component A is from 1 to 1.7 parts regardless of the ingredients thereof. These preferred embodiments are not to be construed as limiting the range of proportions in so far as the scope of the invention is concerned.

The compounding of the thickeners can be done by various processes, some known to the prior art and some new. One new process which I have devised consists in incorporating solid aluminum coconut soap and viscous aluminum naphthenate with kerosene or other high-boiling fuel in a heated mixer. Another is to grind aluminum naphthenate with a sorbent combustible, such as dry wood flour, and mill dry aluminum coconut soap into the mixture; this has the advantage of giving a solid thickening agent very easily dispersed in a hydrocarbon fuel. The preparation of the material in the form of a dry solid also

can be accomplished by methods already known for the precipitation of water-insoluble metal salts from aqueous solutions of the sodium soaps, for example by the process described by A. Minich in British Patent 507,361 (June 14, 1939), or by the process of C. C. Towne (U. S. Patent 2,205,994, June 25, 1940). Thus a convenient procedure consists in preparing an aqueous solution of the sodium salts of the combined acid components containing free alkali, and to add an aqueous solution of aluminum sulfate; this precipitates the thickener as a magma which can be collected by filtration and dried to a granular solid.

In still another process, described below in detail, the mixed aluminum soap thicker is produced in the presence of the fuel which is to be gelled. For example, powdered aluminum coconut soap, with or without admixture with a sorbent combustible such as wood flour or lampblack filler to increase the incendiary efficacy of the gel, is made into a thin slurry with motor gasoline and a concentrated solution of aluminum naphthenate in gasoline is added and the whole briefly mixed. A uniform gel is set up after standing for a few hours.

As an example of a further variation coming within the scope of the present invention, we may cite the preparation of hydrocarbon gels by mixing with the hydrocarbon fuel an aluminum soap selected from the group represented by component A together with a free soap-forming unsaturated fatty acid or cycloparaffinic acid. Typical formulations are as follows:

(6)

7 parts—aluminum soap of coconut acids  
4 parts—Armour's "Neo-Fat 3R" (40% oleic and 60% linoleic acids)  
87 parts—motor gasoline  
2 parts—lampblack

(7)

9 parts—aluminum soap of coconut acids  
5 parts—"Neo-Fat 3R"  
2 parts—lampblack  
84 parts—motor gasoline

These gels are made very easily by briefly stirring the aluminum soap and the filler with gasoline to form a thin slurry and adding the unsaturated acid component. After brief mixing, no further processing is required and a stiff transient gel is set up within a few minutes at ordinary temperature and changes to a stringy permanent gum after about one day. Formulation (6) is well adapted to use in tail ejection bombs, while formulation (7) is distinctly tougher and is recommended for a burster-type bomb where resistance to the shattering action of an explosive is required.

The gels prepared in gasoline (for example, ordinary motor gasoline or gasoline of 11.5 lbs. Reid vapor pressure and 140° F. aniline point) at concentrations of 12 to 13.5% of thickener are very full-bodied and strong and very well adapted to use in explosive type bombs because of their strength and resistance to the shattering action of the burster charge. Gasoline gels containing 8-9% of thickener have considerable body and possess desirable stringiness and extensibility and are well suited for use in bombs of the tail-ejection type or in incendiary hand grenades. Gels in higher boiling fuels, exemplified by kerosene and Stoddard solvent, containing approximately 8% of thickener, constitute particularly effective fillings for hand incendiary units consisting of a combustible container of the plasticized nitrocelulose type, and a thickened oil filling. In gen-

eral, a good effective incendiary gel will result from a mixture consisting from 84 to 92 per cent by weight of gasoline or other light liquid hydrocarbon fuels and from about 8 to 16 per cent by weight of any of the thickening composition disclosed.

We have characterized the gels obtained from our new soaps as to body or apparent viscosity to a limited extent by the falling ball method, and also by the use of a Stoermer viscosimeter equipped with a paddle, as described by Geddes and Dawson in Ind. Eng. 34, 163 (1942), wherein the revolutions per minute are plotted against the load imposed. The average weight required to produce a given rate of shear can be used as a characterization of the degree of body of the gel. A perhaps preferable method is with the use of the Gardner mobilometer, and here a brief indication of body can be given as the load required to produce a fall of 10 cm. in 100 sec.

Another significant characterization is the time required for the dispersion of a thickener in a given fuel to give a mixture from which the particles will not settle on standing. The gelation time is also important, and this can be defined as the total time after mixing during which the gel can be easily poured, for example, through a 60° conical funnel with an outlet of 0.625 inch internal diameter and  $\frac{3}{4}$  inch long. The gel is described as pourable as long as 90% of a 500 g. sample will pass through the funnel in not more than 15 secs.

Another test which I have found useful because it gives a ready over-all index of the body and strength of the gel is designated as the "drag test." The test is made in a 7-ounce screw-capped glass bottle (2 $\frac{1}{4}$ " outer diameter) which is charged with enough gel to give a total weight of 325 g. A plunger, consisting of a 1 $\frac{1}{2}$ " by 4 $\frac{3}{4}$ " strip of 0.03-inch Celluloid with a centered hole  $\frac{1}{8}$ " from one end, is pushed to the bottom of the bottle and this is capped and allowed to stand overnight at 77 $\pm$ 2° C. To make the test, the plunger is attached to a hook at such a height that the bottom of the bottle is 7" above the table top; the bottle is released and the time of fall determined. The plunger with adhering gum is then weighed.

I have also assessed the gels of the present invention with respect to their incendiary efficiency by making burning tests conducted in a draft-free room on a standard structure using wood of a given grade and conditioned in the same way to permit reliable comparisons. The standard structure used in these burning tests is shown in the single figure of the drawing.

It consists of a base A of dry whitewood, with posts B, B' and C, C' of dry hemlock upstanding therefrom. Cross pieces E and D, also of dry hemlock, are screwed between the sets of posts B, B' and C, C', respectively, as shown. The posts B, B' and C, C' are firmly nailed to base A with 3-inch nails forced into previously drilled holes, while the cross pieces E and D are held in place between the posts by 2 $\frac{1}{2}$ -inch, No. 11 flat-headed screws. The different pieces making up the structure have the dimensions shown in the drawing.

The test is made by dispersing a standard sample of 97.3 cc. of incendiary gel from a calibrated grease gun on the base board A and noting the time of burning and determining the amount of wood destroyed by weighing the pieces before and after the test, the charred wood being scraped clean before the final weighing.

It will be evident from an examination of the following examples that the soaps claimed as my invention give gels of admirable characteristics as measured by the various criteria enumerated. 5 It should be clearly understood, however, that the examples given below are illustrative and are not to be construed as in any manner limiting the spirit or scope of the appended claims.

#### EXAMPLE I

10 Gel from:

5% aluminum coconut soap  
5% aluminum naphthenate  
90% gasoline (Esso Extra)

15 The naphthenate is added to the gasoline while this is being circulated through a homogenizer, such as a gear pump. When the naphthenate is dispersed, the coconut soap is added and the temperature is brought to 28° C. by friction from the pump. A satisfactory gum is produced in 20 to 30 minutes and requires little subsequent aging to reach a permanent state. A filler can be added after the naphthenate has dissolved, thereby improving the incendiary efficiency, as shown 20 in the following results of burning tests contained in Table I. An average value obtained with a rubber gel is included, and the comparison shows the superior performance of gels prepared with the present thickener.

30

TABLE I

|                                            | Wood burned, g. | Time of burning |
|--------------------------------------------|-----------------|-----------------|
| 35 6% Crepe Rubber in Esso Extra Gasoline. | 493             | 2 min. 25 sec.  |
| Gel of Example I.                          | 440             | 2 min. 27 sec.  |
| Gel of Example I with 0.5% Lampblack.      | 517             | 4 min.          |
| Gel of Example I with 1% Lampblack.        | 530             | 3 min. 46 sec.  |
| Gel of Example I with 1% Sawdust.          | 546             | 2 min. 40 sec.  |

#### EXAMPLE 2

Gel from:

5% aluminum coconut soap  
3% aluminum naphthenate (Nuodex)  
45 0.5% lampblack  
91.5% gasoline (Esso Extra)

The gel is prepared in the manner of the gel of Example I, and is full bodied and tough, and 50 burning tests gave the values 502 g. and 452 g.

#### EXAMPLE 3

Gel from:

4% aluminum coconut soap  
55 5% aluminum oleate (Shepherd)  
90% gasoline (Esso Extra)  
1% lampblack

The ingredients are mixed in a homogenizer and give a gel of excellent character. A standard 97.3 cc. sample burned for 3 min. and 25 sec. and destroyed 543 g. of wood. The formulation can be varied, for example, by using 4% aluminum coconut soap and 6% aluminum oleate (cyanamid).

#### EXAMPLE 4

Field filling of a bomb with a gel from:

70 2 $\frac{1}{4}$  gals. of a 16% solution of aluminum naphthenate in motor gasoline  
2.1 pounds aluminum coconut soap  
6.9 ounces lampblack  
4 $\frac{1}{2}$  gals. motor gasoline

The aluminum coconut soap and lampblack 75 are stirred into the gasoline to give a fluid slurry

which is poured into the bomb through a funnel. The solution of naphthenate is then added, the bomb is closed with a plug or a burster well, and the contents mixed by brief tumbling. The initial gelation results in a few minutes and a final gel is set up after storage at about 20° C. for 5-6 hours.

EXAMPLE 5

Powdered thickener from:

2.36 lbs. aluminum naphthenate  
1.88 lbs. dried wood flour  
2.36 lbs. aluminum coconut soap

The powdered thickener is prepared by incorporating the aluminum naphthenate into wood flour in a meat grinding machine, milling the mix for 10-15 minutes in a Simpson mixer, adding aluminum coconut soap and milling a few minutes longer. A granular powder results which tends to agglomerate slightly on standing, but it can be loosened and poured readily through a funnel into a bomb charged with gasoline. Gelation takes place a few minutes after mixing the powder with gasoline; and if the loaded bomb is set on its side, a satisfactory gum can be obtained even without tumbling. After 5-6 hours the gum reaches a terminal state and is ready for use. A suitable filling for a bomb consists in 5.95 lbs. of the above powder added to 4 gals. of gasoline in the bomb and followed by an additional 2 gals. of gasoline. Field trials indicate that the gel is tough and resistant to shattering.

The powder above described is an excellent thickener for the filling of frangible hand grenades. For example, the grenade can be stored and shipped without the fuel but charged with the proper amount of the aluminum soap-wood flour powder; at any time prior to use, gasoline can be added and the grenade shaken briefly and allowed to stand for a few minutes for gelation.

The gel as described when submitted to the standard burning test, burns for the unusually long time of 6½ minutes and destroys 645 g. of wood. The stability at both -40° F. and +155° F. is excellent.

EXAMPLE 6

5-lb. charge of aluminum naphthenate is put into a steam-jacketed mixer heated with steam at a pressure of about 5 lbs. and milled until it becomes sticky and doughy (about 5 minutes). A previously prepared suspension of 5 lbs. of aluminum coconut soap in 10 lbs. of diesel fuel, made by adding the powder slowly and paddling it to an even slurry, is poured slowly into the naphthenate in the mill at such a rate as to keep the mix doughy and to avoid a local excess of unmilled fluid. After the addition is complete, the cover is put in place and the mix is milled for 30 minutes, with careful control of the temperature (by occasionally stopping the mill and inserting a thermometer). The gum should reach a temperature of 75-85° C. in 15 minutes, and at the end of 30 minutes it should be at 95-100° C. and not over 100° C. The resulting thickener is a soft gum.

For the preparation of 19.2 lbs. of incendiary gum, 5.7 lbs. of the above thickener is put through a Hobart meat grinder, using a delivery plate having  $\frac{1}{8}$ -inch holes. The issuing stream of soft, spaghetti-like strands is run directly into a 5-gal. tank containing 13.5 lbs. of gasoline which is being circulated by means of a gear pump. After the addition is complete, the mixture is kept circulating for 15-20 minutes, when it becomes thick and fairly well mixed, and it is

then pumped directly into the bomb and allowed to stand for 5-6 hours for the setting up of the final gel.

A standard sample of this gel, which shows excellent stability in the range from -40° F. to +155° F., destroys 588 g. of wood. The gum is more resistant to the shattering action of an explosive than any of those described in the above examples. It gives excellent performance in both 30 lb. and 100 lb. burster-type bombs and also performs well in tail-ejection bombs. The filling operation is simple and adaptable to the plant scale filling of incendiary bombs.

EXAMPLE 7

Thickener prepared from the coprecipitated aluminum soap from:

2 parts coconut fatty acids  
1 part naphthenic acid  
1 part oleic acid

The coprecipitation is carried out by the process of British Patent 507,361, namely by addition of aluminum sulfate solution to a solution of the sodium soaps of the combined acids in the presence of excess alkali at temperatures below the boiling point of water. The precipitated material is collected by filtration and dried in air or in vacuum at temperatures not exceeding 150° F. and with care to avoid any local overheating, due, for example, to the packing of the material in too thick layers. The moisture content of the final product is preferably kept below 2% as determined by the loss in weight on air-drying a sample for 15 hours at 150° ± 5° F.

This thickener is fully soluble in gasoline and kerosene and other hydrocarbon solvents and is easily incorporated into such fuels by brief mixing. The dispersion time and setting time in gasoline, for example, of Reid vapor pressure 11.5 lbs. and aniline point 140° F. is dependent on the size and porosity of the acid particles and can be controlled readily by controlling the character of the solid. Thus a typical sample ground to a rather fine powder showed the dispersion time of  $\frac{1}{4}$  minute and a setting time at which it became unpourable of  $\frac{1}{2}$  minute. When compressed by hand into  $\frac{1}{8}$ " pellets, the respective times were 11 minutes and 60 minutes. As an illustration of the way in which the time for dispersion and setting can be decreased, pellets compressed in the same way but utilizing thickener powder mixed with 1% dried wood flour showed a dispersion of 3 minutes and a setting time of 5½ minutes. The same powder without wood flour when compressed on a roller at 5,000 lbs. per square inch and screened to 8 mesh, showed a dispersion time of 9 minutes and a setting time of 13 minutes.

Gels prepared in the gasoline specified above, using 50 g. of thickener to 366.4 g. of the gasoline, when tested with the Stoermer viscosimeter give values for the revolutions per minute as low as 0.2 at a load of 600 g. When tested after a period of aging at 120° F. for 20 hours, the R. P. M. at a load of 600 g. is not in excess of 3.0. Cooling of the gel at -40° F. and inspection for syneresis on agitation or a tendency to turn brittle, reveals no such shortcomings.

Eight per cent gels of the thickener in the same gasoline, when tested in the Gardner mobilometer after the sample has stood in the tube for four hours at 77° ± 2° F. are found to have apparent viscosities such that the load required to produce a fall of 10 cm. in 100 sec. is not less than 500 g. nor more than 1200 g.

11  
EXAMPLE 8

*Preparation of hydrocarbon gels from aluminum soap of coconut acids and various unsaturated and cycloparaffinic acids*

Gels in gasoline or in kerosene are prepared by mixing the aluminum coconut soap with the fuel, adding the fatty acid component, and agitating the mixture at ordinary temperature for a short time either by stirring or by passing it through a gear pump homogenizer. An initial stiff gel is produced, usually in less than one hour, and changes to a more stringy consistency after standing for about 24 hours.

Table II below lists formulations employing various acid components, including Armour and Company's "Neo-Fat 3R" (40% oleic, 60% linoleic), "Neo-Fat 17" ( $C_{20}$  and  $C_{22}$  unsaturated acids), "Neo-Fat 19" ( $C_{20}$  acid with 3 and 4 double bonds); also oleic acid, the acids of linseed oil, and the cycloparaffinic naphthenic acid. Examination of the data descriptive of the gels will show that the most satisfactory performance is obtained with Neo-Fat 3R and Neo-Fat 19.

TABLE II.—GASOLINE GELS PREPARED WITH ALUMINUM COCONUT SOAP (ACS) AND VARIOUS ACID COMPONENTS AND BINDERS

| No. | Percent ACS | Acid Component, Binder                 | Remarks                                                                                                                                       |
|-----|-------------|----------------------------------------|-----------------------------------------------------------------------------------------------------------------------------------------------|
| 8a  | 5           | 2% Neo-Fat 3R                          | Good at $-40^{\circ}$ C., slightly thin at $52^{\circ}$ C.; burning test 336 g., 1 min. 46 sec.                                               |
| 8b  | 7           | 4% Neo-Fat 3R                          | Stable on cycling at $-40^{\circ}$ and $+52^{\circ}$ C.; good body throughout this range; stringy; burning test: 402 g., 2 $\frac{1}{2}$ min. |
| 8c  | 7           | 4% Neo-Fat 3R<br>12% Lampblack         | Improved incendiary efficiency; burning test: 531 g.                                                                                          |
| 8d  | 9           | 15% Neo-Fat 3R<br>2% Lampblack         | Tough, durable gum, withstands explosion by black powder, stronger than (c).                                                                  |
| 8e  | 7           | 4% Neo-Fat 3R<br>2% Lampblack          | Stronger than (c), slightly less resistant to explosive wave than (d).                                                                        |
| 8f  | 5           | 2% Neo-Fat 19                          | Gelled at $21^{\circ}$ ; very similar to (a); burning test 399 g., 2 min. 30 sec.                                                             |
| 8g  | 5           | 2% Neo-Fat 17                          | Very thick, but rather brittle and jello-like.                                                                                                |
| 8h  | 5           | 2% Oleic Acid                          | Less satisfactory at low and high temperatures.                                                                                               |
| 8i  | 5           | 2% Naphthenic Acid                     | Rather thin gel.                                                                                                                              |
| 8j  | 5           | 12% Naphthenic Acid                    | Full-bodied but rather jello-like.                                                                                                            |
| 8k  | 7           | 14% Linseed oil acids<br>12% Lampblack | Good gel, particularly tough and stringy at $52^{\circ}$ C.                                                                                   |

The amounts of the two components and the ratio between them is of some significance and the formulation is best varied to meet a specific use. Thus the gel No. 8a has a tendency to become thin at elevated temperatures and gives a somewhat low value in the wood burning test. An increase in the total amount of added ma-

EXAMPLE 9  
50 Preparation of hydrocarbon gels with the use of oleic-linoleic acids in combination with various aluminum soaps

The gels listed in Table III are prepared as described in Example 8.

TABLE III.—GASOLINE GELS PREPARED WITH NEO-FAT (N-F) 3R (40% OLEIC, 60% LINOLEIC) AND VARIOUS ALUMINUM SOAPS

| No. | Aluminum Soap  |         | Remarks                                                           |
|-----|----------------|---------|-------------------------------------------------------------------|
|     | Percent N-F 3R | Percent |                                                                   |
| 9a  | 4              | 7       | 50 Lauric, 20 myristic, 10 palmitic, 5 stearic, 15 N-F 3R.        |
| 9b  | 4              | 7       | 55 myristic, 20 palmitic, 10 stearic, 10 N-F 3R, 5 naphthenic.    |
| 9c  | 4              | 7       | 15 naphthenic, 45 myristic, 20 palmitic, 5 stearic, 15 N-F 3R.    |
| 9d  | 4              | 7       | 50 2-Ethylhexoic, 20 myristic, 10 palmitic, 5 stearic, 15 N-F 3R. |
| 9e  | 4              | 7       | 70 myristic, 10 palmitic, 5 stearic, 15 N-F 3R.                   |
| 9f  | 4              | 7       | Hydronaphthalenedicarboxylic acids (Du Pont).                     |

## 13

In this series, the acid component (Neo-Fat 3R) was that found most generally appropriate in the example of Table II. The aluminum soap component is made by a process of precipitation or coprecipitation from an aqueous solution containing free alkali, utilizing the acids and acid mixtures indicated. Example 9a shows that a satisfactory gel can be obtained with a mixture of acids roughly approximating that ordinarily found in the acids of coconut oil. If the lauric acid is omitted as in Example 9b, the heat stability of the gel is definitely less. A considerable increase in the myristic acid to compensate for the absence of lauric acid leads to a gel of less satisfactory character (9e), for it does not possess adequate heat stability. If the lauric acid component is replaced by a mixture of naphthenic and myristic acid (9c), the gel is stringy but lacks body. Replacement of the lauric acid and coconut acids by 2-ethylhexoic acid (9d) results in a gel of generally satisfactory characteristics. Example 9f illustrates the possibilities in the way of employing as the aluminum soap component material entirely of synthetic origin; the mixture of acids used is made by the addition of sodium to naphthalene, followed by carbonation with carbon dioxide. The gel prepared with this soap alone in combination with Neo-Fat 3R is too stringy and brittle to be fully satisfactory, but the combination has great bodying power.

## EXAMPLE 10

*Field filling of a bomb with a gel from aluminum coconut soap, Neo-Fat 3R, lampblack and gasoline*

A three-gallon milk can with calibration markings is filled to the first mark with 3.83 pounds of aluminum coconut soap and 0.85 pound of lampblack is added to the next mark, and the two powders are well mixed. A crimped cover, having a few 1" perforations on one side, is put in place and the container is grasped by a handle running along the side and the contents are shaken into 5.65 gals. of gasoline contained in an eight-gal. metal pail which has suitable calibration markings. During the addition of the powder, the gasoline is stirred with a wooden paddle. A thin, even suspension results and this is poured into the bomb through a large funnel. A 2-qt. screw-capped tin can containing a mixture of Neo-Fat 3R (2.58 pounds) and sufficient gasoline to keep it from solidifying at low temperatures (0.15 gal.) is opened and the contents poured into the bomb. A screw plug is inserted and the bomb is tumbled a few times and let stand at a temperature of 15° C. or higher. Ini-

## 2,606,107.

## 14

## EXAMPLE 11

Thickeners prepared as the coprecipitated aluminum soaps from:

- 5 2 parts—total nut oil split acids  
1 part—naphthenic acid (refined), acid No. 237,  
unsap. 8%.  
1 part—oleic acid

## ANALYSES OF THE NUT OIL ACIDS

|    |                          | Coconut | Babassu | Palm Kernel |
|----|--------------------------|---------|---------|-------------|
| 10 | Acid No.                 | 271.7   | 261.5   | 259.0       |
|    | Sap. No.                 | 270.6   | 260.2   | 258.2       |
| 15 | Titer, ° C.              | 23.5    | 22.4    | 23.1        |
|    | Iod. No.                 | 8.2     | 17.5    | 17.0        |
|    | Unsap. percent           | .26     | .28     | 0.30        |
|    | Probable lauric, percent | 47.1    | 41.9    | 50.0        |

20 The samples were dried to a moisture content of 0.5-2.0%, as determined by the loss in weight on drying at 20-30 mm. pressure at 70° C. for 48 hours. The average ash content is 13.2%, and the average aluminum content, determined by extraction of a petroleum naphtha gel with nitric acid, conversion to the sulfate, precipitation with ammonia, and calcination at 1200° C., is 5.9%. Samples exposed to air for 15 hrs. at 60° C. showed no loss of solubility in hydrocarbon solvents or in gelling efficiency. In Table IV, coconut acid, babassu acid and palm kernel acid, are compared for the stringiness and viscosity which they impart to incendiary gels.

TABLE IV—INSPECTIONS OF 12 PERCENT GELS IN  
35 "STANDARD" GASOLINE (11.5 REID V. P., ANILINE  
POINT 140° F.)

| 40 | Variable Ingredient    | Stringiness and body— |            | Stoermer<br>R. P. M. at<br>650 g. load |                  |
|----|------------------------|-----------------------|------------|----------------------------------------|------------------|
|    |                        | at -40° F.            | at 125° F. | Initial                                | After<br>125° F. |
|    |                        |                       |            |                                        |                  |
| 45 | (11a) Coconut Acid     | ++++                  | ++++       | .092                                   | .11              |
|    | (11b) Babassu Acid     | +++                   | ++++       | .051                                   | .03              |
|    | (11c) Palm kernel Acid | +++                   | ++++       | .043                                   | .03              |

50 The three thickeners of Table IV are all of high quality, and differences between them are of a minor nature. Variations in the naphthenic acid and oleic acid also produce but slight change in the character of the thickener and the gels obtained therefrom. For example, samples of naphthenic acid of acid number ranging from 230 to 243 and containing from 2 to 8% unsaponifiable material can be used with equally satisfactory results.

GELATION OF VARIOUS HYDROCARBON FUELS WITH SOAP 11a  
(TABLE IV)

| Solvent         | Per cent Thick-ener | Gelation Time, Min. | R. P. M./650 g. | Remarks              |
|-----------------|---------------------|---------------------|-----------------|----------------------|
| Gasoline        | 12                  | 1                   | 0.20            | Full-bodied, tough.  |
| Hexane Fraction | 12                  | 9                   | .46             | Slightly thinner.    |
| Isooctane       | 12                  | 25                  | .02             | Rather short.        |
| Benzene         | 12                  | 1.5                 | .06             | Very tough.          |
| Do.             | 8                   | 1.5                 | .35             | Good, tough stringy. |
| Do.             | 6                   | 1.5                 | 200             | Very thin.           |
| Cyclohexane     | 12                  | 2                   | .07             | Very tough.          |
| Do.             | 8                   | 2                   | .15             | Good, tough stringy. |
| Do.             | 6                   | 2                   | 200             | Very thin.           |

tial gelation occurs in  $\frac{1}{4}$  to 1 hour, depending upon the temperature, and the gum becomes stringy and ready for use in 10-15 hours.

It is evident that the time required for gelation varies greatly with structure of the hydrocarbon, and also that with aromatic and cycloparaffinic

hydrocarbons considerably less soap is required to produce a gel of a given viscosity.

EXAMPLE 12

Thickener prepared as the coprecipitated aluminum soap from:

- 2 parts—coconut oil acid  
1 part—unrefined naphthenic acid  
1 part—oleic acid

The soap, obtained as a dry, dark brown powder, has considerable bodying power; for example, a 12% gel in "standard" gasoline is comparable in viscosity with those described above in Example 11 (Stoermer R. P. M./650 g.=0.095). Although suitable for some purposes, the gels from this soap lack strength and are not well adapted to use in bombs and shells. This deficiency is easily recognized from the results of "drag tests" with 13.5% gels. Those from soaps 11a, 11b and 11c of Example 11 show times of fall of 17, 12 and 27 sec., respectively, and the plunger retains an amount of gum in excess of 9 g. With the gel from soap 12 the test bottle falls free in 2 seconds and retains only 2-3 g. of gum. We consider a gel to have passed this test (at  $77 \pm 2^\circ \text{C}$ ) if the time of fall is at least 10 seconds and the weight of sample adhering to the plunger at least 9 g.

EXAMPLE 13

Thickeners prepared as the coprecipitated aluminum soaps from:

- 2 parts—special fatty acid fraction  
1 part—naphthenic acid (refined)  
1 part—oleic acid

In this series variation is made in the saturated fatty acid component by employing a number of commercial fractions from coconut oil acids and from the acids of animal and fish oils. The fractions are described in the following Table V, those found to give the most satisfactory soaps being starred.

TABLE V.—HIGH-LAURIC FATTY ACID FRACTIONS

| No. | Designation | Description | Acid No. | Sap. No. | Titer °C. | Iod. No. |
|-----|-------------|-------------|----------|----------|-----------|----------|
|-----|-------------|-------------|----------|----------|-----------|----------|

FROM COCONUT OIL

|      |                           |                                                                                |       |       |      |      |
|------|---------------------------|--------------------------------------------------------------------------------|-------|-------|------|------|
| 13a* | Weccoline AAAR            | Residue from the stripping of lower acids (10%); contains about 8% glycerides. | 234.0 | 254.5 | 25.6 | 9.2  |
| 13b* | E. F. Drew Special Sample | Total distilled acids plus 7% glycerides.                                      | 233.9 | 268.7 | 23.0 | 7.6  |
| 13c* | Weccoline AB              | Distilled Weccoline AAAR                                                       | 251.2 | 252.6 | 25.4 | 12.7 |
| 13d* | Weccoline AAB             | High lauric cut                                                                | 246.9 | 249.1 | 25.2 | 14.8 |
| 13e* | W. C. Smith               | Lauric and higher acids                                                        | 258.0 | 259.2 | 27.9 | 8.9  |
| 13f* | W. C. Smith               | Lauric-myristic cut                                                            | 268.8 | 268.9 | 31.9 | 0.7  |

FROM ANIMAL OR VEGETABLE OILS

|      |            |                   |       |       |      |     |
|------|------------|-------------------|-------|-------|------|-----|
| 13g* | Neo-Fat 11 | 90% lauric acid   | 279.5 | 279.7 | 37.8 | 1.0 |
| 13h  | Neo-Fat 13 | 90% myristic acid | 248   | 248.2 | 51   | 2.0 |

FROM FISH OILS

|      |                      |                            |       |       |      |      |
|------|----------------------|----------------------------|-------|-------|------|------|
| 13i* | WCS Sperm Oil Cut 1  | 91% Lauric Acid            | 273.3 | 273.0 | 37.2 | 0    |
| 13j* | WCS Sperm Oil Cut 2  | 75% Myristic Acid          | 238.6 | 240.8 | 43.0 | 3.8  |
| 13k  | WCS Sperm Oil Cut 3  | 20% Myristic, 76% palmitic | 220.7 | 224.0 | 49.2 | 7.8  |
| 13l* | WCS Spermaceti Acids | 15% lauric, 32% myristic   | 215.1 | 224.0 | 43.4 | 11.0 |

One characteristic of soaps compounded with acid fractions of lauric acid content higher than the nut oil acids is an increased speed of gelation and setting in hydrocarbon solvents, as is evident from the following Table VI.

TABLE VI.—8½ GELS IN "STANDARD" GASOLINE

| Soap No. | Nature of the Sat'd Fatty Acids | Time in Min. at 77°F. |         |
|----------|---------------------------------|-----------------------|---------|
|          |                                 | Dispersion            | Setting |
| 11a      | Approx. 50% lauric              | 7                     | 17      |
| 13a      | More than 50% lauric            | 1½                    | 1       |
| 13b      | do                              | 1½                    | 5       |
| 13c      | do                              | 2                     | 4       |
| 13e      | do                              | ½                     | 2       |
| 13f      | do                              | ½                     | 1½      |
| 13g      | 90% lauric                      | ½                     | 1½      |
| 13j      | 75% myristic                    | 1½                    | 5       |
| 13l      | lauric-myristic (47%)           | ½                     | ¾       |

As in other instances, the dispersion and setting times can be extended considerably, if desired, by compression of the solid soap to reduce the porosity, and also by increasing the particle size.

Another characteristic of the soaps prepared from saturated acids rich in the lauric component is that the amount of thickener required to produce a given viscosity often can be substantially reduced beyond that observed with the total nut oil acids. This and other characteristics of the soaps in this series are illustrated by the following descriptions:

A freshly prepared 13.5% gel from soap 13a (Weccoline AAAR) in gasoline is somewhat short, but after five days acquires excellent characteristics, being very tough and reasonably stringy and tacky. No breakdown, thinning, or deterioration has been indicated in heating tests conducted at  $66^\circ \text{C}$ . for periods as long as 700 hours. The concentration of thickener can be reduced to 12% (but not lower) and the gum will still meet the specifications for 13.5% gels defined above by the "drag test." With a soap utilizing total coconut oil acid, for example, No. 11a, Example 11, the concentration often can be reduced to 11% but not 10%.

Soaps 13b-f are very similar in general characteristics to that described. Soap 13g prepared from Neo-Fat 11, consisting almost solely of lauric acid, also has unusual bodying power. The 13.5% gel is so full-bodied as to be somewhat

short, and more satisfactory gels can be prepared with less thickening agent. Thus, an 11% gasoline gel more than meets the requirements of the "drag test" (time of fall, 19 sec.) and the specification is still met with a 10% gel.

In comparison with the soap 13g from 90% lauric acid, soap 13h from 90% myristic acid is less satisfactory. The 13.5% gel in gasoline has satisfactory properties at room temperature, but at 66° C. it becomes very weak and runny. In the series of soaps utilizing fish oil acids, a similar superiority of lauric over myristic is observable. Soap 13i, made from a high lauric cut, has high bodying power and is generally somewhat superior to soap 13j in which myristic acid predominates; however, the latter soap, although of slightly inferior quality, is still rated as satisfactory, as is soap 13l wherein a part of the lauric acid content, characteristic of a nut oil acid, is made up by myristic acid. Soap 13k, however, which has a low myristic content and contains no lauric, is definitely less satisfactory.

#### EXAMPLE 14

Thickeners prepared as the coprecipitated aluminum soaps from:

2 parts—coconut oil acid  
1 part—naphthenic acid  
1 part—special acid component

Although oleic acid is abundantly available and is a wholly satisfactory component, a brief survey is recorded herein of the adequacy of various substitute components. The soaps were evaluated by the inspection of 13.5% gasoline gels at room-temperature, -40° C. and 66° C., and the conclusions may be summarized as follows in Table VII:

TABLE VII

| Spec. Acid Component      | Iod. No. | Evaluation of Gel                          |
|---------------------------|----------|--------------------------------------------|
| Cottonseed oil acid.....  | 90-105   | Very thick, but short and crumbly.         |
| Soya bean oil acid.....   | 122      | Generally satisfactory.                    |
| Corn oil acid.....        | 95-115   | Very thick, but short and brittle.         |
| Linseed oil acid.....     | 179-209  | Good, stringy gel; stability questionable. |
| Neo-Fat 3R.....           | 140      | Excellent gel.                             |
| Armour's Animal Acid..... | 50-70    | Good above -10° C., syneresis at -40° C.   |

#### EXAMPLE 15

Preparation of a gel suitable for burning annual weed seeds from:

75 parts—Stoddard solvent or kerosene  
25 parts—gasoline  
1.5-2.5 parts—aluminum soap, Example 7

The soap is stirred with the mixture of fuels until the particles are solvated sufficiently so they will not settle. After standing at ordinary temperature overnight, the gel is suitable for use. More hydrocarbon fuel is added if required to make the gel fluid enough to pour freely, for example through  $\frac{1}{16}$ -inch perforations in the screw cap of a dispensing container. Gels of this character are particularly suitable for application by spraying on crabgrass or other weeds for the purpose of extermination by the burning of the seeds.

It will be realized from the nature of the invention that a number of substitutions and modifications will be apparent to those skilled in the art without departing from the scope of this invention. Accordingly, it is intended that all matter described and set forth hereinbefore shall

be given the broadest construction consistent with the state of the prior art.

What is claimed as new is:

1. A composition of matter adapted to thicken light liquid hydrocarbon fuels into incendiary gels comprising in parts by weight approximately 1 to 1.7 parts of the aluminum soap of fatty acids found in coconut oil, and approximately one part of aluminum naphthenate.
2. A composition of matter adapted to thicken light liquid hydrocarbon fuels into incendiary gels comprising in parts by weight approximately one part of the aluminum soap of fatty acids found in coconut oil, and approximately 1 to 1.25 parts of aluminum oleate.
3. An incendiary gel comprising from about 84% to about 92% by weight of gasoline thickened with from about 8% to about 16% by weight of a composition comprising in parts by weight approximately 1 to 1.7 parts of aluminum soap of fatty acids found in coconut oil, and approximately one part of aluminum naphthenate.
4. An incendiary gel comprising from about 84% to about 92% by weight of gasoline thickened with from about 8% to about 16% by weight of a composition comprising in parts by weight approximately one part of aluminum soap of fatty acids found in coconut oil, and approximately 1 to 1.25 parts of aluminum oleate.
5. A composition of matter adapted to thicken light liquid hydrocarbon fuels into incendiary gels comprising in parts by weight approximately 1 to 1.7 parts of the hydroxy aluminum soap of fatty acids found in coconut oil and approximately 1 part of hydroxy aluminum naphthenate.
6. A composition of matter adapted to thicken light liquid hydrocarbon fuels into incendiary gels, comprising in parts by weight approximately 1 part of the hydroxy aluminum soap of the fatty acids found in coconut oil, and approximately 1 to 1.25 parts of hydroxy aluminum oleate.
7. A composition of matter adapted to thicken light liquid hydrocarbon fuels into incendiary gels comprising in parts by weight approximately 1 to 2.5 parts of an aluminum soap of a saturated fatty acid fraction having from 8 to 14 carbon atoms per acid molecule, and approximately 1 to 1.25 parts of at least one member of the group consisting of soap-forming naphthenic acid, soap-forming unsaturated fatty acids having from 17 to 22 carbon atoms per acid molecule, and the aluminum soaps of said group of soap-forming acids.
8. A composition of matter adapted to thicken light liquid hydrocarbon fuels into incendiary gels comprising in parts by weight approximately 1 to 1.7 parts of an aluminum soap of a saturated fatty acid fraction having from 8 to 14 carbon atoms per acid molecule and approximately one part of an aluminum soap of naphthenic acid.
9. A composition of matter adapted to thicken light liquid hydrocarbon fuels into incendiary gels comprising in parts by weight approximately one part of an aluminum soap of a saturated fatty acid fraction having from 8 to 14 carbon atoms per acid molecule and approximately 1 to 1.25 parts of an aluminum soap of oleic acid.
10. A composition of matter adapted to thicken light liquid hydrocarbon fuels into incendiary gels comprising in parts by weight approximately one part of an aluminum soap of coconut oil acids and 1.25 parts of an aluminum soap of oleic acid.

11. A composition of matter adapted to thicken light liquid hydrocarbon fuels into incendiary gels comprising in parts by weight approximately 1.5 to 2.5 parts of an aluminum soap of a saturated fatty acid fraction having from 8 to 14 carbon atoms per acid molecule and approximately one part of a mixture of unsaturated fatty acids having 17 to 22 carbon atoms per acid molecule.

12. A composition of matter adapted to thicken light liquid hydrocarbon fuels into incendiary gels comprising in parts by weight approximately 1.5 to 2.5 parts of an aluminum soap of a saturated fatty acid fraction having from 8 to 14 carbon atoms per acid molecule and approximately one part of a mixture of oleic and linoleic acids.

13. A composition of matter, in powder form, adapted to thicken light liquid hydrocarbon fuels into incendiary gels comprising in parts by weight approximately 1 to 2.5 parts of an aluminum soap of a saturated fatty acid fraction having from 8 to 14 carbon atoms per acid molecule and approximately 1 to 1.25 parts of at least one member of the group consisting of soap-forming naphthenic acid, soap-forming unsaturated fatty acids having from 17 to 22 carbon atoms per acid molecule and the aluminum soaps of said group of soap-forming acids and a finely divided combustible sorbent material of the class consisting of comminuted carbon and comminuted wood.

14. An incendiary gel comprising from about 84 to about 92% by weight of a light liquid hydrocarbon fuel thickened with from about 8% to about 16% by weight of a composition comprising in parts by weight approximately 1 to 2.5 parts of an aluminum soap of a saturated fatty acid fraction

having from 8 to 14 carbon atoms per acid molecule, and approximately 1 to 1.25 parts of at least one member of the group consisting of soap-forming naphthenic acid, soap-forming unsaturated fatty acids having from 17 to 22 carbon atoms per acid molecule, and the aluminum soaps of said group of soap-forming acids.

15. An incendiary gel comprising from about 84 to about 92% by weight of a light liquid hydrocarbon fuel thickened with a composition comprising in parts by weight approximately 1 to 2.5 parts of an aluminum soap of a saturated fatty acid fraction having from 8 to 14 carbon atoms per acid molecule, and approximately 1 to 1.25 parts of at least one member of the group consisting of soap-forming naphthenic acid, soap-forming unsaturated fatty acids having from 17 to 22 carbon atoms per acid molecule, and the aluminum soaps of said group of soap-forming acids and a finely divided combustible sorbent material of the class consisting of comminuted carbon and comminuted wood.

LOUIS F. FIESER.

#### REFERENCES CITED

The following references are of record in the file of this patent:

#### UNITED STATES PATENTS

| Number    | Name             | Date          |
|-----------|------------------|---------------|
| 123,683   | Dennis           | Feb. 13, 1872 |
| 488,223   | Rogers           | Dec. 20, 1892 |
| 1,936,632 | Lededer          | Nov. 28, 1933 |
| 2,264,353 | Zimmer et al.    | Dec. 2, 1941  |
| 2,343,736 | Beerbower et al. | Mar. 7, 1944  |
| 2,365,037 | Zimmer et al.    | Dec. 12, 1944 |
| 2,390,609 | Minich           | Dec. 11, 1945 |